

3,296,134

**MINERAL LUBRICATING OIL CONTAINING BIS-PHENOL, DETERGENT AND PHOSPHITE ADDITIVE**

Duk Hi Lee, Berkeley, Calif., assignor to Shell Oil Company, New York, N.Y., a corporation of Delaware  
No Drawing. Filed Apr. 30, 1964, Ser. No. 363,976  
4 Claims. (Cl. 252—46.7)

This invention relates to new and improved mineral 10 lubricating oil compositions containing ashless polymeric detergents.

It is known that phenolic compounds and particularly alkylated bisphenols as described in U.S. Patents 2,807,653 and 2,944,086 are good oxidation inhibitors for lubricating oils, greases, rubbers, waxes, and the like. The art also teaches that these bisphenols form synergistic 15 antioxidant mixtures with certain classes of diaryl acid phosphates or organo-2-thiaphosphono compounds such as dodecyl-2-thiameethylphosphonic acid and esters thereof.

Although it has been observed that benefits are imparted to lubricating oils by addition of bisphenols or mixtures of these bisphenols and pentavalent phosphorous-containing compounds as mentioned with respect to oxidation stability and wear inhibition, it has been found that the addition of such additive mixtures to mineral lubricating oils containing certain types of ashless polymeric detergents results in a decrease of detergent life, resulting in dirty engines in a relatively short period of engine operating time, particularly when the engine is operating at elevated temperatures and pressures or under "stop-and-go" driving conditions.

It has now been discovered that the detergent life of mineral lubricating oils containing ashless polymeric detergents as will be hereinbelow described can be greatly increased by addition of a minor amount of an additive mixture comprising (A) an alkylated bisphenol having the general formula



where Y is a methylene radical or sulfur, X is a halogen, preferably a middle halogen (Cl or Br), R is a tertiary alkyl radical of from 4-8 carbon atoms, m is an integer of 1-3, preferably 2, and n is an integer of zero or 1 and (B) an organic phosphite having the formula



where Z is oxygen and/or sulfur, R' is an aryl or alkaryl radical having 6-18, preferably 6-12 carbon atoms and the sum of x and y is 3 and such that x is at least 2 and y can be zero or 1 and preferably such that x is 3 and y is zero.

The alkylated bisphenols represented by Formula I include alkylated bisphenol sulfides such as bis(2,5-dipentyl-4-hydroxyphenyl)-sulfide, bis(2,5-di-hexyl-3-hydroxyphenyl)sulfide, bis(2-methyl-5-tertiary-butyl-4-hydroxyphenyl)sulfide, bis(2-methyl-5-tertiarybutyl-6-hydroxyphenyl)sulfide and particularly bis(3-tertiarybutyl-5-methyl-2-hydroxyphenyl)sulfide.

The alkylated bisphenols having a methylene bridge, include bis(2,3-di-tertiarybutyl-4-hydroxyphenyl)methane, bis(2,5-di-tertiarybutyl-4-hydroxyphenyl)methane, bis(2,6-di-tertiarybutyl-4-hydroxyphenyl)methane, bis(3,5-di-tertiaryoctyl-4-hydroxyphenyl)methane, bis(3-tertiarybutyl-5-tertiaryoctyl-4-hydroxyphenyl)methane,

and especially bis(3,5-di-tertiarybutyl-4-hydroxyphenyl)methane. The halogen containing bisphenols are illustrated by bis(2-chloro-5-tertiarybutyl-4-hydroxyphenyl)methane, bis(2-bromo-5-tertiarybutyl-4-hydroxyphenyl)methane, bis(2-chloro-5-tertiarybutyl-4-hydroxyphenyl)sulfide and mixtures thereof.

The organic phosphites of Formula II and preferably phosphites having the formula



where R'' is an aryl radical, preferably a monoaryl radical are illustrated by the following examples: diaryl acid phosphites such as diphenyl, ditolyl, dicresyl, di-tertiarybutylphenyl, diocetylphenyl, tertiarybutylmethylphenyl acid phosphites and their thio derivatives; triaryl phosphites, e.g. triphenyl, tritolyl or tricresyl phosphites, and their thio derivatives such as triphenyl, tricresyl or tolyl thio-phosphites and mixtures thereof.

The additive mixture is used in minor amounts each of from 0.01% to 2%, preferably between 0.1% and 0.5% mole.

The particularly preferred additive mixtures on a mole percent basis which are illustrative of the present invention include:

- 25 (Ia) Tritolyl phosphite (0.15%) and bis(3,5-di-tertiarybutyl-4-hydroxyphenyl)methane (0.15%)
- (IIa) Tritolyl thiophosphite (1.0%) and bis(3,5-di-tertiarybutyl-4-hydroxyphenyl)methane (0.15%)
- (IIIa) Triphenyl phosphite (0.5%) and bis(3,5-di-tertiarybutyl-4-hydroxyphenyl)methane (0.1%)

The oil-soluble polymeric detergents which are present in mineral lubricating oils of the present invention and whose detergent life is improved and increased include 35 oxygen- or oxygen and nitrogen-containing polymeric detergents.

The nitrogen-containing polymeric detergents are copolymers of monomers having polymerized linkages and containing nitrogen-containing groups which may be amide 40 or amido groups. They may be derived from polymerizable monomers containing primary, secondary or tertiary (the latter two are preferred) amino nitrogen, including heterocyclic amino or amido nitrogen-containing substances, having an ethylenically unsaturated polymerizable group.

45 These detergent polymers may be obtained by polymerizing vinyl substituted heterocyclic nitrogen-containing substances such as vinyl pyridine, vinyl picoline and vinyl quinoline, vinyl pyrrolidone or vinyl arylamines, such as paraaminostyrene, or polyamines prepared by reacting polymeric epoxy compounds with ammonia or primary or secondary amines, with polymerizable unsaturated alcohols, acids or esters, such as acrylates and methacrylates of long chain fatty acids, and the like. The preferred polymeric amino or amido compounds are those containing tertiary amine groups and particularly those containing heterocyclic amino groups

50 such as obtained by copolymerizing a polymerizable heterocyclic nitrogen base compound with a polymerizable unsaturated material free of heterocyclic nitrogen-containing radicals such as are described in British patent specification 760,554 and U.S. Patents 2,839,512 and 2,889,282. The copolymers include: (A) copolymer of stearyl methacrylate, and 2-methyl-5-vinyl pyridine; (B)

55 copolymer of stearyl methacrylate, lauryl methacrylate and 2-methyl-5-vinyl pyridine; and those which contain additional C<sub>1-4</sub> alkyl methacrylates in the polymer, such as (C) copolymers of stearyl methacrylate, lauryl methacrylate, methyl methacrylate and 2-methyl-5-vinyl pyridine; and similar copolymers in which the methyl methac-

rylate is replaced by butyl methacrylate and the 2-methyl-5-vinyl pyridine is replaced by 5-ethyl-2-vinyl pyridine; or (D) copolymer of lauryl methacrylate and N-vinyl pyrrolidone or similar copolymers as described in the British Patent 808,664 and mixtures thereof. Acrylate N-vinyl pyrrolidone copolymers, e.g. N-vinyl pyrrolidone and lauryl methacrylate can be of varying molecular weights. Other suitable polymeric amines are (E) copolymers of lauryl methacrylate and diethylaminoethylmethacrylate (note U.S. Patent 2,737,496).

Particularly preferred detergent polymers are Acryloid 917 and 966 (copolymers of N-vinyl pyrrolidone and lauryl methacrylate in the molecular weight range of 4,000 to 1,000,000) or the copolymers of vinyl pyridine and mixtures of dissimilar methacrylate esters, such as copolymers (B) or (C) prepared by the methods described in U.S. patents mentioned above and having molecular weight in the range of 450,000 and 850,000 as determined by the light scattering method.

The oxygen-containing detergents include copolymers of  $C_{8-18}$  alkyl acrylates and  $\omega$ -hydroxy alkyl methacrylates, e.g., (F) copolymer of stearyl methacrylate, lauryl methacrylate and 2-hydroxyethyl methacrylate. Other examples of suitable copolymers are those described in U.S. Patents 2,800,453 and 3,033,828. These polymers are present in the oil in amounts ranging from about 1% to about 10%, preferably from about 1.5% to about 5% by weight.

The mineral lubricating oil base may be derived from a variety of petroleum base stocks and are preferably paraffinic and/or naphthenic in character; they may also contain substantial proportions of hydrocarbons having aromatic character. The viscosity may vary within wide limits so that the oils may belong, for example, to SAE classes 5W, 10W, 20W, 20, 30, 40, 50, 60, or 70. Suitable oils may be derived from highly paraffinic crudes in which case distillation and/or dewaxing may be sufficient to provide a suitable base stock; chemical or selective solvent treatment may be used if desired, but is preferably kept to a minimum for economic reasons. Mixed-base crudes and even highly aromatic crudes which contain paraffinic hydrocarbons also provide suitable oil base stocks after refining by well-known techniques such as the separation of distillate fractions of suitable boiling range followed by solvent extraction with selective solvents, for example, furfural or phenol, to provide raffinate fractions, dewaxing, and chemical treatment, for example, sulfuric acid treatment.

Illustrative compositions of the present invention are as follows:

Composition (a):

|                                                                                                                  |         |
|------------------------------------------------------------------------------------------------------------------|---------|
| Mixture (Ia), percent mole                                                                                       | 0.3     |
| Copolymer (C) stearyl methacrylate/lauryl methacrylate/2 - methyl - 5 - vinyl pyridine (MW=800,000), percent wt. | 1.5     |
| Mineral lubricating oil                                                                                          | Balance |

Composition (b):

|                                                                                     |         |
|-------------------------------------------------------------------------------------|---------|
| Mixture (Ia), percent mole                                                          | 0.3     |
| Copolymer (D) lauryl methacrylate and N-vinyl pyrrolidone (MW=450,000), percent wt. | 5       |
| Mineral lubricating oil                                                             | Balance |

Composition (c):

|                             |         |
|-----------------------------|---------|
| Mixture (IIa), percent mole | 1.15    |
| Copolymer (C), percent wt.  | 5       |
| Mineral lubricating oil     | Balance |

Composition (d):

|                                  |         |
|----------------------------------|---------|
| Mixture (IIIa), percent mole     | 0.6     |
| Copolymer (C), percent wt.       | 1.5     |
| Dicresyl phosphate, percent wt.  | 0.04    |
| Tricresyl phosphate, percent wt. | 0.8     |
| Mineral lubricating oil          | Balance |

Composition (e):

|                            |         |
|----------------------------|---------|
| Mixture (Ia), percent mole | 0.3     |
| Copolymer (F), percent wt. | 1.5     |
| Mineral lubricating oil    | Balance |

In the LS-3 Cadillac Engine Test operated under the following conditions: 400 repeating cycles of 15 minutes each, comprising 1 minute at 90° F. jacket temperature, 10 minutes at 135° F. jacket temperature and 2500 r.p.m. and 4 minutes at 190° F. jacket temperature at 3200 r.p.m., using high sulfur (1%) fuel, the results were as follows: Composition (a) ran for over 100 hours at which time the engine was clean, free of sludge and corrosion and otherwise in excellent condition. When Composition (a) was modified by removing the tritolyl phosphite and this modified phosphorus-free composition identified as Composition (X) was used in the LS-3 test and visible sludge formation was noted at end of 40 hours and engine had to be stopped. Essentially the same results are obtainable using Compositions (b), (c), or (d) of the present invention as were obtained with Composition (a). On the other hand when, in composition (X) the bis(3,5-di-tertiary-butyl - 4-hydroxyphenyl)methane was substituted with equal amount (0.3% mole) of tritolylphosphite to form Composition (Y) and engine tested (LS-3 condition), operation of the engine had to be terminated at the end of 20 hours because of heavy sludge formation. For purpose of clarity the formulation of Compositions (X) and (Y) are as follows:

Composition (X):

|                                                                                                                  |         |
|------------------------------------------------------------------------------------------------------------------|---------|
| Bis(3,5-di-tert-butyl - 4-hydroxyphenyl)methane, percent mole                                                    | 0.3     |
| Copolymer (C) stearyl methacrylate/lauryl methacrylate/2 - methyl - 5 - vinyl pyridine (MW=800,000), percent wt. | 1.5     |
| Mineral lubricating oil                                                                                          | Balance |

Composition (Y):

|                                                                                                                  |         |
|------------------------------------------------------------------------------------------------------------------|---------|
| Tritolyl phosphate, percent mole                                                                                 | 0.3     |
| Copolymer (C) stearyl methacrylate/lauryl methacrylate/2 - methyl - 5 - vinyl pyridine (MW=800,000), percent wt. | 1.5     |
| Mineral lubricating oil                                                                                          | Balance |

Additive mixture of the present invention can be also used to improve fuels, fuel oils, greases, asphalts, oil emulsions and the like.

We claim as our invention:

1. A mineral lubricating oil composition comprising a major amount of mineral lubricating oil and from about 1% to about 10% of a copolymer of 2-hydroxyethyl methacrylate and a mixture of lauryl and stearyl methacrylates and from about 0.01% to about 2% each of (A) an alkylated bisphenol having the formula



where Y is a radical selected from the group consisting of  $-\text{CH}_2-$  and  $-\text{S}-$ , X is a halogen, R is a tertiary alkyl radical of 4 to 8 carbon atoms and m and n are integers such that m is at least 1 and n can be zero and (B) an organic phosphite having the formula



where Z is an element selected from the group consisting of oxygen and sulfur, R' is an aryl radical and x+y equal 3 and y is at least 2.

2. The composition of claim 1 where Y is  $-\text{CH}_2-$ , n is zero, Z is oxygen, and y is zero and x is 3.

3. A mineral lubricating oil composition comprising a major amount of mineral lubricating oil and from about 1% to about 10% of a copolymer of 2-hydroxyethyl methacrylate and a mixture of lauryl and stearyl methacrylates and from about 0.01% to about 2% each of

5

bis(3,5-di-tertiary-butyl-4 - hydroxyphenyl)methane and tritolyl phosphite.

4. A mineral lubricating oil composition comprising a major amount of mineral lubricating oil and from about 1% to about 10% of a copolymer of 2-hydroxyethyl methacrylate and a mixture of lauryl and stearyl methacrylates and from about 0.01% to about 2% each of bis(3,5-di-tertiarybutyl - 4-hydroxyphenyl)methane and ditolyl phosphite.

6

|           |         |                  |       |          |
|-----------|---------|------------------|-------|----------|
| 2,758,091 | 8/1956  | Webber           | ----- | 252-49.9 |
| 3,100,749 | 8/1963  | Wittner et al.   | ----- | 252-49.9 |
| 3,115,465 | 12/1963 | Orloff et al.    | ----- | 252-49.9 |
| 3,215,631 | 11/1965 | Henderson et al. | ----- | 252-49.9 |

5

## OTHER REFERENCES

|           |        |                |
|-----------|--------|----------------|
| 845,255   | 8/1960 | Great Britain. |
| 1,299,534 | 6/1962 | France.        |

10 DANIEL E. WYMAN, *Primary Examiner.*W. H. CANNON, *Assistant Examiner.*

## References Cited by the Examiner

## UNITED STATES PATENTS

2,188,943 2/1940 Evers ----- 252-46.6